

# United States Patent [19]

Fischer et al.

[11] 3,860,522

[45] Jan. 14, 1975

[54] **SYNTHETIC LUBRICANTS RESISTANT TO SHEAR AND COLD**

[76] Inventors: **Diether Fischer**, 7 Im Sandgarter, Wachenheim; **Paul Hornberger**, 12 In den Ziegelgaerten; **Willy Wolf**, 8 Alwin-Mitlasch-Platz, both of Ludwigshafen, all of Germany

[22] Filed: **Apr. 6, 1971**

[21] Appl. No.: **131,796**

[30] **Foreign Application Priority Data**

Apr. 14, 1970 Germany ..... 2017744

[52] U.S. Cl. .... **252/56 S, 252/59**

[51] Int. Cl. .... **C10m 1/28**

[58] Field of Search. .... **252/56 S, 59**

[56] **References Cited**

UNITED STATES PATENTS

2,610,948 9/1952 Morway et al. .... 252/56 S

|           |        |                     |          |
|-----------|--------|---------------------|----------|
| 2,746,925 | 5/1956 | Garber et al. ....  | 252/59   |
| 2,891,084 | 6/1959 | Alm et al. ....     | 252/56 S |
| 3,098,042 | 7/1963 | Morway et al. ....  | 252/59   |
| 3,271,311 | 9/1966 | Morway et al. ....  | 252/59   |
| 3,329,613 | 7/1967 | Fischer et al. .... | 252/59   |

Primary Examiner—Daniel E. Wyman

Assistant Examiner—Y. H. Smith

Attorney, Agent, or Firm—Johnston, Keil, Thompson & Shurtleff

[57] **ABSTRACT**

Shear-resistant and cold-resistant synthetic lubricants consisting of a mixture of esters of branched-chain dicarboxylic acids of from 16 to 22 carbon atoms and aliphatic alcohols of less than 6 carbon atoms with polymers of butenes having a molecular weight of from 1,200 to 4,500, the ester portion being from 10 to 95% by weight and the polymer portion from 90 to 5% by weight.

4 Claims, No Drawings

## SYNTHETIC LUBRICANTS RESISTANT TO SHEAR AND COLD

This invention relates to shear-resistant and cold-resistant synthetic lubricants.

In industry there is an ever-increasing demand for lubricating oils showing good flow at low temperatures yet possessing adequate viscosity at higher temperatures. The lubrication of engines and gears is carried out with multi-grade oils based on mineral lubricating oils and influenced in their viscosity/temperature characteristic by the addition of polymers, V.I. improvers, such that the classifying features of the SAE oils as laid down in German Standard Specifications DIN 51511 and 51512 for winter and summer use respectively are combined in a single oil.

However, the performance of such multi-grade oils based on a mineral oil is highly unsatisfactory for a number of reasons. If the amount of V.I. improvers - e.g. polyacrylates or polymethacrylates - added is to remain within tolerable limits, the use of additional use of paraffin base oils is inevitable. Cooling of the oils causes the pour point to be reached as a result of crystallization of solid paraffins. Although the pour point may be lowered by the addition of pour point depressants, the viscosities in the range between the turbidity point and pour remain higher than anticipated for the liquid phase due to the precipitation of crystallizable paraffin components; distinct differences may be observed between the low-temperature viscosity calculated by extrapolation of viscosity measurements made at higher temperatures by the method described in German Standard Specification DIN 51563 and the low-temperature viscosity as actually measured. This increased viscosity greatly restricts the range of application of these oils.

Moreover, such multi-grade oils containing V.I. improvers are not stable to the action of shearing forces encountered under operating conditions. The resulting decrease in viscosity and reduction of the viscosity index impairs the viscosity/temperature characteristic and the original multi-grade character of the oil is lost. Finally, the addition of V.I. improvers modifies the stability of the oil, and such modification must be counteracted by increasing the addition of inhibitors and materials having a cleaning effect on the interior of the engine.

Lubricants based on dicarboxylates, for example non-substituted or alkyl-substituted adipates and sebacates, have been known in the art for a number of years. The combined use of ester oils and mineral oils for lubricating purpose has also been known for many years.

Furthermore, in special lubricating applications requiring pure lubricants based on hydrocarbons and free from foreign matter, it is known to use liquid polymers of butenes or isobutylene. However, these polymers are unduly volatile compared with mineral oils of the same viscosity and their flash point characteristic is unsatisfactory. The said polymer oils have a viscosity/temperature characteristic which is approximately the same as that of mineral oils.

We have now found that excellent shear-resistant and cold-resistant synthetic lubricants are obtained by mixing esters of branched-chain dicarboxylic acids of from 16 to 22 carbon atoms and aliphatic alcohols of less than 6 carbon atoms with polymers of butenes having a molecular weight of from 1,200 to 4,500, the ester

portion being from 10 to 95% by weight and the polymer portion being from 90 to 5% by weight.

Esters which may be used in the present invention are, in particular, esters of heptadecanodic acid with 5 propanol, n-butanol or isobutanol or mixtures of these butanols. Other suitable esters are those of alkyl-substituted adipic or sebacic acids of from 16 to 22 carbon atoms, for example decyladipic acid, dodecyladipic acid, octylsebacic acid, dibutylsebacic acid and 10 dihexylsebacic acid with ethanol, propanol or butanol as the alcohol component. Polymers which may be used according to the invention in admixture with the said esters are those having a molecular weight of from 1,200 to 4,500 as measured by the Staudinger method.

15 They are light to heavy oils having viscosity/temperature characteristics similar to those of mineral lubricating oils. The polymers are prepared by known methods and may, if desired, be hydrogenated before blending with the esters.

20 Particularly suitable mixtures for use in the present invention are those of from 45 to 80% by weight of ester with from 55 to 20% by weight of a polymer having a molecular weight of from 2,500 to 4,000 and mixtures of from 20 to 50% by weight of ester with from 25 80 to 50% by weight of a polymer having a molecular weight of from 1,200 to 3,000.

25 The previously known viscosity/temperature-improved lubricants based on mineral lubricating oils or mixtures of mineral lubricating oils with ester oils have distinct disadvantages:

30 To achieve the usual multi-grade properties it is necessary to add a V.I. improver. This gives these multi-grade oils their wellknown susceptibility to shearing forces, which results in a reduction of viscosity in use.

35 The low-temperature viscosities are unfavorably influenced, i.e. raised, by the precipitation of paraffin from the mineral oil portion. The measured viscosities do not satisfy the viscosity/temperature relationship given in German Standard Specification DIN 51563.

40 This restricts the range of utility of the oils at low temperatures.

45 The stability of esters is impaired when they are blended with a mineral base oil. This is shown in stability tests using the test strip apparatus by Wolf. For example, a di-n-butyl heptadecanodicarboxylate achieves the high rating of 8.5 when tested in this apparatus without any additive, whilst the rating achieved by a conventional mineral base oil without any additive is 5.0. A mixture of the ester with the same base oil (with no further additive) in a ratio of 1:1 also achieves a value of 5.0. The better stability of the ester oil is lost when the latter is mixed with a mineral base oil.

50 However, by mixing dicarboxylates with polymers of butenes according to the present invention multi-grade oils are provided which are completely stable to shear and which satisfy the V/T relationship given in German Standard Specification DIN 51 563 down to very low temperatures, e.g. -40°C. In addition, the mixtures of the invention show superior aging stability to comparable lubricants containing mineral oil.

### EXAMPLE 1

55 63 parts of di-n-butyl heptadecanodicarboxylate are mixed with 37 parts of a poly(isobutylene) having an average molecular weight of 3,000 as measured by the Staudinger method. There is thus obtained a clear, pale, stable oil having the following properties:

|               | Number of passes through Bosch nozzle |       |       |       |       |       |
|---------------|---------------------------------------|-------|-------|-------|-------|-------|
|               | 0                                     | 1     | 2     | 5     | 10    | 20    |
| cSt at 37.8°C | 68.89                                 | 62.20 | 61.27 | 60.85 | 60.00 | 59.46 |
| cSt at 98.9°C | 10.78                                 | 9.38  | 9.15  | 8.98  | 8.86  | 8.76  |
| V.I.          | 136                                   | 130   | 128   | 126   | 126   | 125   |

|                          | according to<br>DIN 51562 | Extrapolated<br>according<br>to DIN 51563 |
|--------------------------|---------------------------|-------------------------------------------|
| Viscosity at 98.9°C      | 10.13 cSt                 | —                                         |
| 37.8°C                   | 64.95 cSt                 | —                                         |
| -17.8°C                  | 2220                      | about 2200                                |
| Viscosity index          | 134                       |                                           |
| SAE class                | 10W/30                    |                                           |
| Pour point               | -57°C                     |                                           |
| Flash point              | 236°C                     |                                           |
| Noack test (250°C)       | 12%                       |                                           |
| Conradson carbon residue |                           |                                           |

The oil thus obtained has excellent cold viscosities. By comparison, the viscosities, as measured by German Standard DIN 51562, of comparable commercial oils based on a mineral oil are much higher at low temperatures and differ from the values obtained by extrapolation:

|                   | Viscosity<br>according to<br>DIN 51562 | Extrapolated<br>according<br>to DIN 51563 |
|-------------------|----------------------------------------|-------------------------------------------|
| Comparative oil A |                                        |                                           |
| 98.9°C            | 10.78 cSt                              | —                                         |
| 37.8°C            | 68.89 cSt                              | —                                         |
| -17.8°C           | 3150 cSt                               | 2200 cSt                                  |
| -30°C             | no longer measurable                   | 7500 cSt                                  |
| Comparative oil B |                                        |                                           |
| 98.9°C            | 10.45 cSt                              | —                                         |
| 37.8°C            | 67.83 cSt                              | —                                         |
| -17.8°C           | 3050                                   | 2300                                      |
| -30°C             | 50000                                  | 8500                                      |
| -40°C             | no longer measurable                   | 30,000 cSt                                |

Comparative oil A is a 10W/30 multi-grade oil prepared by adding 4.8% of a V.I. improver and 5.2% of a detergent/inhibitor combination to a mineral lubricating oil. It has a viscosity index of 136.

The comparative oil B is also a 10W/30 multi-grade oil which contains, however, in addition to the mineral lubricating oil, 23% of di-n-butyl heptadecanodicarboxylate as oil component. In this case the amount of V.I. improver added is 3% and that of the detergent/inhibitor combination is 6%. The viscosity index is 134.

The oil of the invention as described in this Example also possesses absolute stability to shear. Testing of the shear resistance by the method of forcing the oil through a Bosch-Diesel injection nozzle at a pressure of 55 200 atmospheres shows no reduction of the viscosity or of the viscosity index:

|               | Number of passes through Bosch nozzle |       |       |       |       |       |
|---------------|---------------------------------------|-------|-------|-------|-------|-------|
|               | 0                                     | 1     | 2     | 5     | 10    | 20    |
| cSt at 37.8°C | 64.95                                 | 65.30 | 64.32 | 64.57 | 65.43 | 64.91 |
| cSt at 98.9°C | 10.13                                 | 10.11 | 10.11 | 10.16 | 10.13 | 10.10 |
| V.I.          | 134                                   | 134   | 135   | 135   | 134   | 134   |

The comparative oil A, tested under the same conditions, shows a distinct loss of viscosity and reduction of the viscosity index:

A stability test using the test strip apparatus gave the following results:

|                                         | Rating     |
|-----------------------------------------|------------|
| 63% di-n-butyl heptadecanodicarboxylate | 8.5        |
| 37% poly(isobutylene) mol.wt. 3,000     |            |
| 63% di-n-butylheptadecanodicarboxylate  |            |
| 37% mineral lubricating oil Solvent     |            |
| Neutral (2.5°E/50°C)                    | 5.0 to 5.5 |
| 100% mineral lubricating oil Solvent    |            |
| Neutral (2.5°E/50°C)                    | 5.0        |

The oil of the invention as described in Example 1 has the rating 8.5. This rating is excellent for an oil not containing any additives for improving the detergent-dispersant characteristic. The rating of commercial HD oils of the test strip apparatus is between 8.0 and 10.0, whilst mineral base oils achieve ratings of approximately 5. If the esters are not mixed with poly(isobutylene) as proposed by the invention but with a conventional mineral base oil, the rating achieved is much the same as that of the mineral base oil alone.

#### EXAMPLE 2

50 parts of di-n-butyl heptadecanodicarboxylate are mixed with 50 parts of poly(isobutylene) having a molecular weight of 3,200. The mixture has the properties of a 20W/50 multi-grade oil having excellent cold viscosities and shear resistance:

|                     | Measured   | Extrapolated |
|---------------------|------------|--------------|
| Viscosity at 98.9°C | 18.08 cSt  |              |
| 37.8°C              | 152.53 cSt |              |
| -17.8°C             | 8300 cSt   | 8000 cSt     |
| -30°C               | 29100 cSt  | 32500 cSt    |
| V.I.                | 125        |              |
| SAE class           | 20W/50     |              |
| Pour point          | -55°C      |              |

Following 20 passes through a Bosch nozzle in the shear test the oil has the following values:

|                     |           |
|---------------------|-----------|
| Viscosity at 98.9°C | 18.05 cSt |
| 37.8°C              | 153.03    |
| -17.8°C             | 125       |
| V.I.                | 20W/50    |

A comparable commercial 20W/50 oil prepared by mixing a mineral base oil with a V.I. improver and a detergent/inhibitor combination, has the following data:

|              | Measured                             | Extrapolated                      |
|--------------|--------------------------------------|-----------------------------------|
| Viscosity at | 98.9°C<br>37.8°C<br>-17.8°C<br>-30°C | 17.94 cSt<br>no longer measurable |
| V.I.         | 129                                  | 25000 cSt                         |
| SAE class    | 20W/50                               |                                   |
| Pour point   | -40°C                                |                                   |

In the shear test, the viscosity of the oil fell to the following values after 20 passes through the Bosch nozzle:

|              |                  |                         |
|--------------|------------------|-------------------------|
| Viscosity at | 98.9°C<br>37.8°C | 15.14 cSt<br>124.33 cSt |
| V.I.         | 123              |                         |
| SAE class    | 20W/40           |                         |

### EXAMPLE 3

30 parts of di-isobutyl heptadecanodicarboxylate are mixed with 70 parts of poly(isobutylene) having a molecular weight of 1,500. The mixture has the viscosity characteristic of a highly cold-resistant and shear-resistant SAE 80/90 multi-grade oil:

|              | Measured                    | Extrapolated                    |
|--------------|-----------------------------|---------------------------------|
| Viscosity at | 98.9°C<br>37.8°C<br>-17.8°C | 17.80 cSt<br>171.0<br>12700 cSt |
| V.I.         | 117                         | 13200 cSt                       |
| SAE class    | 80/90                       |                                 |

These data remain unchanged after 20 passes through a Bosch nozzle.

The oils produced by mixing esters and poly(isobutylene)

as proposed by the invention may be used as such for lubricating purpose; or conventional lubricant additives may be added, such as those for improving the detergent characteristic, the attrition characteristic, the resistance to oxidation and the pressure resistance, to extend the range of application of the oils. However, the addition of V.I. improvers is not necessary.

The lubricants of the invention may be advantageously used in a variety of lubricating applications. For example they may be used as engine oils, gear oils, hydraulic oils, ATF oils, shock-absorber oils, turbine oils and oils for lubricating aeroturbines.

We claim:

1. Shear-resistant and cold-resistant synthetic lubricants consisting essentially of a mixture of esters of branched-chain dicarboxylic acids of from 16 to 22 carbon atoms and aliphatic alcohols of less than 6 carbon atoms with homopolymers of butenes having a molecular weight of 2,500 to 4,000, said esters being 45 to 80% by weight of said mixture and said homopolymers being 55 to 20% by weight of said mixture.

2. Shear-resistant and cold-resistant synthetic lubricants consisting essentially of a mixture of esters of branched-chain dicarboxylic acids of from 16 to 22 carbon atoms and aliphatic alcohols of less than 6 carbon atoms with homopolymers of butenes having a molecular weight of 1,200 to 3,000, said esters being 20 to 50% by weight said mixture and said homopolymers being 80 to 50% by weight of said mixture.

3. Lubricants as claimed in claim 2 wherein said ester component is the ester of heptadecanedioic acid with n-butanol, isobutanol or mixtures thereof.

4. Lubricants as claimed in claim 1 wherein said ester component is the ester of heptadecanedioic acid with n-butanol, isobutanol or mixtures thereof.

\* \* \* \* \*

UNITED STATES PATENT AND TRADEMARK OFFICE  
CERTIFICATE OF CORRECTION

PATENT NO. : 3,860,522

DATED : Jan. 14, 1975

INVENTOR(S) : Diether Fischer, Paul Hornberger, Willy Wolf

It is certified that error appears in the above-identified patent and that said Letters Patent are hereby corrected as shown below:

In the heading, third line in the section of the Inventors, delete "Zlegelgaerten" AND substitute --Ziegelgaerten--.

In the heading, fourth line in the section of the Inventors, delete "Mitlasch" and substitute --Mittasch--.

Column 6, line 29, delete "weight said mixture" and substitute--weight of said mixture--.

Signed and Sealed this  
fourth Day of May 1976

[SEAL]

Attest:

RUTH C. MASON  
Attesting Officer

C. MARSHALL DANN  
Commissioner of Patents and Trademarks